

March 4, 1930.

H. G. WALKER

1,749,008

INSULATING MATERIAL

Filed Aug. 31, 1927



Fig. 1.



Fig. 2



Fig. 3.

Fig. 4.



Inventor  
Howard G. Walker  
by A. Schattom Atty.

## UNITED STATES PATENT OFFICE

HOWARD GEORGE WALKER, OF LA GRANGE, ILLINOIS, ASSIGNOR TO WESTERN ELECTRIC COMPANY, INCORPORATED, OF NEW YORK, N. Y., A CORPORATION OF NEW YORK

## INSULATING MATERIAL

Application filed August 31, 1927. Serial No. 216,625.

This invention relates generally to insulating materials, and more particularly to water-resistant, insulating materials.

Many insulating materials have sufficient water repellent properties to permit their use when they are subjected only to atmospheric moisture, or to more severe conditions for short periods of time, but due to their water absorbent properties most of them are unsuited for use where they are continuously exposed to extremely humid conditions or are submerged in water.

The present invention has for its object the provision of an insulating material having desirable insulating characteristics and also having the property of retarding the passage of moisture therein so that the effective life of the insulating material in the presence of moisture is materially lengthened.

In accordance with the general features of the invention, an insulating material of any suitable type, such as a rubber compound, is prepared and finely divided particles of a non-corrosive material having a large surface area capable of retaining moisture are dispersed throughout the rubber compound. The resulting composition may then be applied to the article to be insulated, such as an electrical conductor, and vulcanized thereon.

It is believed that the invention will be clearly understood from the following detailed description of specific embodiments of the invention taken in conjunction with the accompanying drawing, in which

Fig. 1 is a fragmentary longitudinal view of a portion of a cable embodying the invention;

Fig. 2 is a transverse sectional view thereof taken on line 2—2 of Fig. 1;

Fig. 3 is a fragmentary longitudinal view of another type of cable embodying the invention, and

Fig. 4 is a transverse sectional view thereof taken on line 4—4 of Fig. 3.

Numerous experiments have shown that practically all electrical insulating materials absorb water to a greater or a lesser degree and, in view of this fact, insulating compositions of the type which form the subject matter of this invention have been developed to

provide compositions which have a retarded rate of water absorption and which consequently have an increased effective life in the presence of moisture.

Figs. 1 and 2 of the drawing illustrate a portion of an electric cable in which the insulating material has been utilized to protect the conductor therein from moisture. Referring now to those figures, the numeral 10 designates an electrical conductor around which a plurality of conductors 11—11 are arranged in the form of helices. Surrounding the conductors 10 and 11—11 is a layer of insulating material 12 comprising a rubber compound 13 throughout which are dispersed particles 14—14 of a non-corrosive material, such as silica gel, having a large surface area capable of retaining moisture. This layer of insulating material is in turn surrounded by another layer 15 of a suitable insulating and waterproof material, such as a rubber compound, which is substantially impervious to water and the layer 15 is covered by a strip of fabric 16 wound spirally therearound, which may in turn be covered with additional protective layers if desired.

A suitable composition for use in the layer 12 is as follows:

|                     |           |    |
|---------------------|-----------|----|
| Smoked sheet rubber | 50 to 55% | 80 |
| Hard rubber dust    | 18 to 23% |    |
| Silica gel          | 15 to 5%  |    |
| Zinc oxide          | 7.75%     |    |
| Litharge            | 6.25%     |    |
| Sulphur             | 2%        |    |
| Paraffin            | 1%        | 85 |

This composition may be applied to the conductors by extrusion or by any of the other usual methods and vulcanized thereon in any suitable manner well known in the art.

Should a cable of the type disclosed in Figs. 1 and 2 be exposed to extremely humid conditions or be submerged in water, a small quantity of moisture would slowly penetrate through the insulating material 15 and would enter the insulating layer 12 surrounding the conductors 10 and 11—11. However, instead of the moisture penetrating the layer of insulating material 12 and coming directly into contact with the conductors 11—11 and 10,

the moisture which has penetrated through the insulating layer 15 will be taken up by the particles 14-14 and retained thereby, since each of the particles 14-14 of silica gel or other similar non-corrosive material has an extremely large surface area capable of retaining moisture. These particles will continue to absorb and retain any moisture which penetrates through the insulating layer 15 and thereby prevent the moisture from reaching the conductors surrounded by the insulating layer 12 until the particles 14-14 have become substantially saturated with water. It will thus be seen that although the insulating material forming the subject matter of this invention does not completely inhibit the passage of moisture therethrough, it materially lengthens the period of time required for moisture to penetrate from the outside of the layer of material to the inner portions thereof.

Another type of cable employing the insulating material is disclosed in Figs. 3 and 4, in which the numerals 20 and 21 indicate a pair of electrical conductors which are surrounded and separated by an insulating material 22 of the same type as the insulating material forming the layer 12 in the cable illustrated by Figs. 1 and 2, and the insulating material 22 is in turn enclosed within a lead sheath 23. A cable of the type illustrated in Figs. 2 and 3 is especially useful for power purposes in mines, etc., where it would be subjected to extreme conditions of moisture. Although the lead sheath 23 will under ordinary circumstances exclude moisture from the interior of the cable, if the sheath should be broken the water absorbing particles dispersed throughout the layer 22 would absorb and retain any moisture which enters the breach for a considerable length of time and would thereby delay the complete failure of the cable.

It is, of course, to be understood that the invention is not to be limited to the specific composition disclosed hereinbefore but is limited only by the spirit and scope of the annexed claims. For example, another composition which is suitable for uses similar to those described above is as follows:

|    |                     |           |
|----|---------------------|-----------|
| 50 | Smoked sheet rubber | 49%       |
|    | Powdered silica     | 30 to 35% |
|    | Silica gel          | 10 to 5%  |
|    | Zinc oxide          | 3%        |
| 55 | Litharge            | 5%        |
|    | Sulphur             | 2%        |
|    | Paraffin            | 1%        |

In fact, the invention embraces any insulating material having properties similar to those of rubber compounds throughout which is dispersed a material having a large absorptive surface area capable of retaining moisture. The insulating material may consist of a rubber compound, gutta percha, balata, mixtures thereof, or any other materials having simi-

lar insulating and protective properties, and the term "insulating material" as used hereinbefore and in the annexed claims is intended to include all of the above mentioned materials.

What is claimed is:

1. An insulating material comprising approximately 50 to 55% rubber, 18 to 23% hard rubber dust, 15 to 5% silica gel, 7.75% zinc oxide, 6.25% litharge, 2% sulphur, and 1% paraffin.

2. An insulating material comprising approximately 50 to 55% rubber, 25.75 to 30.75% fillers, 15 to 5% silica gel, 8.25% vulcanizing ingredients, and 1% paraffin.

In witness whereof, I hereunto subscribe my name this 17th day of August A. D., 1927.

HOWARD GEORGE WALKER.

70

75

80

35

90

95

100

105

110

115

120

125

130